

# United States Patent [19]

Niebylski

[11] 4,052,171

[45] Oct. 4, 1977

[54] **FUEL COMPOSITIONS AND ADDITIVE MIXTURES CONTAINING METHANETRICARBOXYLATES FOR REDUCING EXHAUST GAS CATALYST PLUGGING**

[75] Inventor: **Leonard M. Niebylski, Birmingham, Mich.**

[73] Assignee: **Ethyl Corporation, Richmond, Va.**

[21] Appl. No.: **643,090**

[22] Filed: **Dec. 22, 1975**

## Related U.S. Application Data

[63] Continuation-in-part of Ser. No. 584,141, June 5, 1975, Pat. No. 3,950,145.

[51] Int. Cl.<sup>2</sup> ..... **C10L 1/16**

[52] U.S. Cl. ..... **44/68; 44/70; 252/386**

[58] Field of Search ..... **44/68, 70; 252/386; 260/485 R, 537 R**

## [56] References Cited

### U.S. PATENT DOCUMENTS

|           |        |                        |           |
|-----------|--------|------------------------|-----------|
| 1,995,615 | 3/1935 | Jaeger .....           | 44/70     |
| 2,747,979 | 5/1956 | Thompson .....         | 44/70     |
| 3,130,017 | 4/1964 | Shapiro et al. .....   | 44/68     |
| 3,328,440 | 6/1967 | Shapiro et al. .....   | 44/68     |
| 3,798,266 | 3/1974 | Bottaccio et al. ..... | 260/537 R |

Primary Examiner—Daniel E. Wyman

Assistant Examiner—Mrs. Y. Harris-Smith

Attorney, Agent, or Firm—Donald L. Johnson; Robert A. Linn; Willard G. Montgomery

## [57] ABSTRACT

Gasoline compositions and additive mixtures of esters of 1,1,2-ethane tricarboxylic acid, in amount sufficient to alleviate the plugging of certain catalysts being used in an engine exhaust system to lower the amount of undesirable constituents in exhaust gas from an engine being operated on gasoline containing a cyclopentadienyl manganese antiknock.

40 Claims, No Drawings

**FUEL COMPOSITIONS AND ADDITIVE  
MIXTURES CONTAINING  
METHANETRICARBOXYLATES FOR REDUCING  
EXHAUST GAS CATALYST PLUGGING**

**CROSS-REFERENCE TO RELATED  
APPLICATION**

This application is a Continuation-in-Part of copending application Ser. No. 584,141, filed June 5, 1975, now U.S. Pat. No. 3,950,145 the entire disclosure of which is incorporated herein by reference.

**BACKGROUND OF THE INVENTION**

Cyclopentadienyl manganese compounds are excellent antiknocks in gasoline used to operate internal combustion engines. These manganese compounds have proved to be especially beneficial in solving some of the problems present when low-lead or lead-free gasolines are used with internal combustion engines. Use of such compounds as antiknocks is described in U.S. Pat. No. 2,818,417; U.S. Pat. No. 2,839,552; and U.S. Pat. No. 3,127,351, incorporated herein by reference. Not only are these compounds effective antiknock compounds, but it has also been found that they do not adversely affect the activity of oxidation metal catalysts used to decrease the amount of undesirable constituents in engine exhaust gas. Under some operating conditions it has been found that, although the manganese antiknocks do not lessen the activity of the exhaust gas catalyst, they can interact in some manner at the surface of the catalyst bed leading to a reduction in the size of the openings into the bed thereby causing an increase in exhaust backpressure and a decrease in the effective life of said catalysts. The present invention provides a simple effective means of alleviating this problem.

It has been previously suggested that the addition of triethyl citrate to gasoline mixes containing organomanganese antiknocks tends to reduce catalyst plugging. The use of triethyl citrate, however, has proved to be of rather limited success in reducing the plugging problem, especially at higher temperatures.

**SUMMARY**

According to the present invention, the useful life of an exhaust gas catalyst in an exhaust system of an engine operating on gasoline containing a cyclopentadienyl manganese antiknock is greatly increased by providing new additive fluids and gasoline compositions which contain an amount of an ester of 1,1,2-ethane tricarboxylic acid or gasoline soluble derivative thereof sufficient to alleviate plugging of the exhaust gas catalyst.

**DESCRIPTION OF THE PREFERRED  
EMBODIMENTS**

The essence of the present invention resides in reducing the plugging of oxidation metal catalytic apparatus for purifying exhaust gases of internal combustion engines which burn a gasoline containing an organomanganese compound. This reduction in plugging is effected by the addition of esters of 1,1,2-ethane tricarboxylic acid, its gasoline soluble salts, or other gasoline soluble derivatives to the gasoline. Accordingly, a preferred embodiment is a gasoline suitable for use in an internal combustion engine and containing an amount of organomanganese compound, preferably a cyclopentadienyl manganese tricarbonyl, sufficient to increase its antiknock effectiveness, and also containing an amount

sufficient to prevent plugging of the catalyst of esters of 1,1,2-ethane tricarboxylic acid, its gasoline soluble salts, or other gasoline soluble derivatives.

A further embodiment of the present invention is a gasoline additive fluid composition comprising an organomanganese compound, preferably a cyclopentadienyl manganese tricarbonyl, and most preferably methylcyclopentadienyl manganese tricarbonyl, in an amount sufficient to improve the antiknock characteristics of the gasoline and esters of 1,1,2-ethane tricarboxylic acid, its gasoline soluble salts and other gasoline soluble derivatives, preferably the mono-, di-, and triesters of 1,1,2-ethane tricarboxylic acid, and most preferably the triesters of 1,1,2-ethane tricarboxylic acid, in an amount sufficient to reduce catalyst plugging.

Since the invention also embodies the operation of an internal combustion engine in a manner which results in reduced plugging of the catalyst, a still further embodiment is a method of operating an internal combustion engine using a gasoline containing an organomanganese, preferably a cyclopentadienyl manganese tricarbonyl, and most preferably methylcyclopentadienyl manganese tricarbonyl antiknock in a manner which results in substantial reduction in the plugging of the catalyst, said method comprising (a) supplying to the fuel induction system of said engine a gasoline containing an organomanganese antiknock and a gasoline soluble solution of the esters of 1,1,2-ethane tricarboxylic acid, its salts, or other gasoline soluble derivatives, (b) mixing said gasoline with air, (c) inducing the mixture into the combustion chambers of said engine, (d) compressing said mixture, (e) igniting said compressed mixture, and (f) exhausting the resultant combustion products which have a reduced plugging effect on the catalyst through said catalyst.

Liquid hydrocarbon fuels of the gasoline boiling range are mixtures of hydrocarbons having a boiling range of from about 80° F. to about 430° F. Of course, these mixtures can contain individual constituents boiling above or below these figures. These hydrocarbon mixtures contain aromatic hydrocarbons, saturated hydrocarbons and olefinic hydrocarbons. The bulk of the hydrocarbon mixture is obtained by refining crude petroleum by either straight distillation or through the use of one of the many known refining processes, such as thermal cracking, catalytic cracking, catalytic hydroforming, catalytic reforming, and the like. Generally, the final gasoline is a blend of stocks obtained from several refinery processes. The final blend may also contain hydrocarbons made by other procedures such as alkylate made by the reaction of C<sub>4</sub> olefins and butanes using an acid catalyst such as sulfuric acid or hydrofluoric acid.

Preferred gasolines are those having a Research Octane Number of at least 85. A more preferred Research Octane Number is 90 or greater. It is also preferred to blend the gasoline such that it has a content of aromatic hydrocarbons ranging from 10 to about 60 volume percent, an olefinic hydrocarbon content ranging from 0 to about 30 volume percent, and a saturate hydrocarbon content ranging from about 40 to 80 volume percent, based on the whole gasoline.

In order to obtain fuels having properties required by modern automotive engines, a blending procedure is generally followed by selecting appropriate blending stocks and blending them in suitable proportions. The required octane level is most readily accomplished by employing aromatics (e.g., BTX, catalytic reformate or

the like), alkylate (e.g., C<sub>6,9</sub> saturates made by reacting C<sub>4</sub> olefins with isobutane using a HF or H<sub>2</sub>SO<sub>4</sub> catalyst), or blends of different types.

The balance of the whole fuel may be made up of other components such as other saturates, olefins, or the like. The olefins are generally formed by using such procedures as thermal cracking, catalytic cracking and polymerization. Dehydrogenation of paraffins to olefins can supplement the gaseous olefins occurring in the refinery to produce feed material for either polymerization or alkylation processes. The saturated gasoline components comprise paraffins and naphthenes. These saturates are obtained from (1) virgin gasoline by distillation (straight run gasoline), (2) alkylation processes (alkylates) and (3) isomerization procedures (conversion of normal paraffins to branched chain paraffins of greater octane quality). Saturated gasoline components also occur in so-called natural gasolines. In addition to the foregoing, thermally cracked stocks, catalytically cracked stocks and catalytic reformates contain saturated components.

The classification of gasoline components into aromatics, olefins and saturates is well recognized in the art. Procedures for analyzing gasolines and gasoline components for hydrocarbon composition have long been known and used. Commonly used today is the FIA analytical method involving fluorescent indicator adsorption techniques. These are based on selective adsorption of gasoline components on an activated silica gel column, the components being concentrated by hydrocarbon type in different parts of the column. Special fluorescent dyes are added to the test sample and are also selectively separated with the sample fractions to make the boundaries of the aromatics, olefins and saturates clearly visible under ultraviolet light. Further details concerning this method can be found in "1969 Book, of ASTM Standards," January 1969 Edition, under ASTM Test Designation D 1319-66T.

The motor gasolines used in formulating the improved fuels of this invention generally have initial boiling points ranging from about 80° to about 105° F. and final boiling points ranging from about 380° to about 430° F. as measured by the standard ASTM distillation procedure (ASTM D-86). Intermediate gasoline fractions boil away at temperatures within these extremes.

From the standpoint of minimizing atmospheric pollution to the greatest extent possible, it is best to keep the olefin content of the fuel as low as can be economically achieved as olefins reportedly give rise to smog-forming emissions, especially from improperly adjusted vehicular engines. Accordingly, in the preferred base stocks of this invention the olefin content will not exceed about 10 volume percent and the most particularly preferred fuels will not contain more than about 5 percent olefins. Table I illustrates the hydrocarbon type makeup of a number of particularly preferred fuels for use in this invention.

TABLE I

Hydrocarbon Blends of Particularly Preferred Base Fuels

| Fuel | Volume Percentage |         |           |
|------|-------------------|---------|-----------|
|      | Aromatics         | Olefins | Saturates |
| A    | 35.0              | 2.0     | 63.0      |
| B    | 40.0              | 1.5     | 58.5      |
| C    | 20.0              | 2.5     | 77.5      |
| D    | 33.5              | 1.0     | 65.5      |
| E    | 36.5              | 2.5     | 61.0      |

TABLE I-continued

Hydrocarbon Blends of Particularly Preferred Base Fuels

| Fuel | Aromatics | Olefins | Saturates |
|------|-----------|---------|-----------|
| F    | 43.5      | 1.5     | 55.0      |
| G    | 49.5      | 2.5     | 48.0      |

10 It is also desirable to utilize base fuels having a low sulfur content as the oxides of sulfur tend to contribute an irritating and choking character to smog and other forms of atmospheric pollution. Therefore, to the extent it is economically feasible, the fuel will contain not more than about 0.1 weight percent of sulfur in the form of conventional sulfur-containing impurities. Fuels in which the sulfur content is no more than about 0.02 weight percent are especially preferred for use in this invention.

20 Normally the gasoline to which this invention is applied is lead-free or substantially lead-free, although small amounts of organolead additives usually employed to give fuels of improved performance quality such as tetraalkyllead antiknocks including tetramethyllead, tetraethyllead, physical or redistributed mixtures

25 of tetramethyllead and tetraethyllead, and the like may be present therein. The gasoline may also contain anti-knock quantities of other agents such as cyclopentadienyl nickel nitrosyl, N-methyl aniline, and the like. Anti-knock promoters such as tert-butyl acetate may be included. The gasoline may further contain blending agents or supplements such as methanol, isopropanol, t-butanol and the like. Antioxidants such as 2,6-di-tert-butylphenyl, 2,6-di-tert-butyl-p-cresol, phenylenediamines such as N,N'-di-sec-butyl-p-phenylenediamine, N-isopropylphenylenediamine, and the like, may be present. Likewise, the gasoline can contain dyes, metal deactivators, or other types of additives recognized to serve some useful purpose in improving the gasoline quality.

30 Cyclopentadienyl manganese tricarbonyls are known antiknocks and their preparation and use are described in U.S. Pat. No. 2,818,417; U.S. Pat. No. 2,839,552; and U.S. Pat. No. 3,127,351. An important antiknock of this type is methylcyclopentadienyl manganese tricarbonyl. The amount of the cyclopentadienyl manganese tricarbonyl added to the gasoline should be an amount adequate to increase its antiknock effectiveness. This has generally been found to be in the range of from about 0.005 to 10 grams per gallon of manganese as a cyclopentadienyl manganese tricarbonyl. A preferred range is from about 0.05 to 6 gm (grams) of manganese per gallon as a cyclopentadienyl manganese tricarbonyl.

35 A more preferred range is from about 0.05 to about 0.25 grams of manganese per gallon, and a most preferred range is from about 0.05 to about 0.125 grams of manganese per gallon as methylcyclopentadienyl manganese tricarbonyl.

40 The exhaust gas purification apparatus are well known and generally employ an oxidation catalytic metal such as platinum, rhodium, palladium, or iridium or combinations thereof. Some examples of catalytic converter units are described in U.S. Pat. No. 3,441,381 and U.S. Pat. No. 3,692,497. The essential elements of 45 such units consist of a catalytic reactor formed by an enlarged cylindrical-frustoconical housing having an inlet port and an outlet port. Located within the housing is a catalyst bed which is a honeycomb alumina-

50

55

60

65

magnesia-silica monolithic ceramic-supported platinum catalyst.

In order to obtain rapid warmup required for catalyst activation, the catalytic reactor is preferably located proximate to the engine exhaust outlet. By proximate is meant that it is close enough that the catalyst bed is rapidly heated to "light off" or activation temperature. The exhaust gas temperature required to accomplish this is dependent upon the nature of the catalyst. Noble metal catalysts containing at least some noble metal such as platinum, palladium or mixtures thereof, activate at lower exhaust temperatures, e.g., 350°-500° F. However, in order to ensure activation, the catalytic reactor is preferably located such that the inlet exhaust temperature is above about 1,000° F. and more preferably above about 1,400° F. during normal engine cruise conditions. It is also at temperatures above about 1,400° F. and at concentrations of manganese of and above 0.25 gms per gallon that the cyclopentadienyl manganese antiknocks are most likely to plug the catalyst and, hence, it is under these conditions that the present invention is most useful. With concentrations of manganese of less than 0.25 gms per gallon and at temperatures under 1,400° F. plugging of the catalyst does not occur.

In tests run with the aforementioned catalytic converters containing monolithic ceramic supports it has been found that plugging occurs by "spikes" forming on the entrance surface of the cordierite ceramic. These form a network which essentially traps large manganese particles and caps the entrance to the monolithic core.

As stated above, the exhaust gas catalyst unit uses a honeycomb, monolithic ceramic, supported platinum catalyst. These are made by coating a corrugated ceramic structure with an activated alumina and a palladium compound. The preferred ceramics are made using alumina-silica, magnesia-alumina-silica (e.g., cordierite) or mixtures thereof. Palladium can be used in place of platinum, and since these elements generally occur in nature together, it is sometimes preferred to use mixtures of platinum and palladium.

The utility of the invention in alleviating plugging with noble metal catalysts suggests its use with other catalysts if an undesirable amount of plugging is noted. Many non-noble metals have been suggested for exhaust gas catalyst. Examples of other catalytic metals include V, Cr, Mn, Fe, Co, Ni, Cu, Zn, Zr, Na, Mo, Ru, Rh, Ag, W, Re, Os, Ir, Pb, Ba, and the like. These are generally used in an oxide form. They may be used individually or in various groupings such as Cu-Cr, Cu-Cr-V, Cu-Pd, Ni-Cr and the like. They may be supported on the above monolithic ceramic support or on any other of numerous well-known catalyst supports such as granular, pelletized, or extruded alumina, silica, silicalumina, zirconia, magnesia, alumina-magnesia and the like.

The preferred antiplugging agents of the present invention have the general formula



wherein R is independently selected from hydrogen, hydrocarbyl radicals of up to 20 carbon atoms, and substituted hydrocarbyl radicals of up to 20 carbon atoms. For purposes of this invention a hydrocarbyl radical can be defined as an organic group solely composed of hydrogen and carbon atoms. Some nonlimiting

representative examples of hydrocarbyl radicals are alkyl, cycloalkyl, alkenyl, aralkyl, alkaryl, and aryl.

Examples of alkyl groups represented by the R group in the above general formula are methyl, ethyl, n-propyl, isopropyl, n-butyl, isobutyl, sec-butyl, tert-butyl, n-amyl, and the various positional isomers thereof, and likewise the corresponding straight and branched chain isomers of hexyl, heptyl, octyl, nonyl, decyl, undecyl, dodecyl, and the like.

When said R groups are cycloalkyl groups, they may be cyclopropyl, cyclobutyl, cyclopentyl, cyclohexyl, cycloheptyl, cyclooctyl, cyclononyl, cyclodecyl, cycloundecyl, cyclododecyl, and the like. They may also be such cycloaliphatic groups as  $\alpha$ -cyclopropyl-ethyl,  $\alpha$ -cyclobutyl-propyl,  $\beta$ -cyclobutyl-propyl, and similar alkyl derivatives of the higher cycloalkyls.

The R groups in the above general formula may also be alkyenyl groups such as ethenyl, 1-propenyl, 2-propenyl, isopropenyl, 1-butenyl, 2-butenyl, 3-butenyl, and the corresponding branched-chain isomers thereof as for example, 1-isobut enyl, 2-isobut enyl, 2-sec-butenyl, including 1-methylene-2-propenyl, and the various isomers or pentenyl, hexenyl, heptenyl, octenyl, nonenyl, decenyl, undecenyl, and dodecenyl, including 3,3-dimethyl-1-butenyl, 2,3-dimethyl-1-butenyl, 2,3-dimethyl-2-butenyl, 2,3-dimethyl-3-butenyl, 1-methyl-1-ethyl-2-propenyl, and the like.

When said R groups are alkaryl groups, they may be tolyl, 2,3-xylyl, 2,4-xylyl, 2,5-xylyl, 2,6-xylyl, 3,4-xylyl, 3,5-xylyl; o, m, and p-cumanyl, mesityl, o, m, and p-ethylphenyl, 2-methyl-1-naphthyl, 3-methyl-1-naphthyl, 4-methyl-1-naphthyl, 5-methyl-2-naphthyl, 6-methyl-3-naphthyl, 7-methyl-1-naphthyl, 8-methyl-4-naphthyl, 1-ethyl-2-naphthyl, and its various positional isomers and the like.

Examples of aryl groups which may be present in the above general formula are phenyl, naphthyl, and the like.

When said R groups are aralkyl groups, they may be benzyl, phenylethyl, 1-phenylpropyl, 2-phenylpropyl, 3-phenylpropyl, 1- and 2-isomers of phenylisopropyl, 1-, 2-, and 3-isomers of phenylbutyl, and the like.

The substituted hydrocarbyl radicals are hydrocarbyl radicals which contain substituents such as halogen, hydroxyl, carboxyl, alkoxy carbonyl, amino, or amide radicals. Thus, the three R groups may contain the same or different substituents or any one R group may contain one or more of said radicals substituted thereon.

As mentioned above, the R groups may be halogen substituted. Thus, chlorine, bromine, iodine, and fluorine may be substituted on the alkyl, cycloalkyl, alkenyl, alkaryl, aryl, and aralkyl groups which are present. Non-limiting examples of such substituted groups are chloromethyl, chloroethyl, bromoethyl, 2-fluoro-1,2-dibromoethyl, 1-iodopropyl, 2-fluoropropyl, 1-chlorobutyl, 2-bromobutyl, 2-iodo-2-methylpropyl, 1-chloropentyl, 3-fluoro-2-methylbutyl, 3-iodo-2-methylbutyl, 1-chloro-2,2-dimethylpropyl, 2-chloroheptyl, 3-fluorononyl, 1-chlorododecyl, and the like. Examples of halogenated cycloalkyl groups are chlorocyclopropyl, chlorocyclohexyl, 1,2-dichlorohexyl, bromocyclobutyl, iodocyclohexyl, and the like.

Examples of halogen-substituted alkenyl groups are bromoethenyl, chloroethenyl, iodoethenyl, 1-bromodecetyl, and the like.

Examples of halogenated alkaryl groups are chloro-o-tolyl, chloro-p-tolyl, chloro-m-tolyl, 2-bromo-3,4-xylyl,

4-bromo-2,3-xylyl, 5-bromo-2,4-xylyl, 2-bromo-4,5-xylyl, o, m- and p-tolyl, 3-bromomesityl, chloro(methyl)-1-naphthyl, iodo(ethyl)-1-naphthyl, all positional isomers of the above, and the like.

Examples of halogen substituted aryl groups are bromophenyl, 2-bromo-1-naphthyl, 3-bromo-1-naphthyl and all positional isomers thereof, 2,4-dibromophenyl, 2,3-dibromophenyl, 2,5-dibromophenyl, 2,3,4,5-tetrabromophenyl, 2,3,5,6-tetrabromophenyl, penta-bromophenyl, all isomers of chlorophenyl, and all isomers of multichlorophenyl: 2-chloro-1-naphthyl and the remaining isomers thereof: 2,3-dichloro-1-naphthyl, 2,4-dichloro-1-naphthyl and the remaining positional isomers of dichloronaphthyl, 2,3,4,5-tetrachloro-1-naphthyl.

Amine groups may also be substituted on the R groups. Some non-limiting illustrative examples of R groups containing amine substituents are aminomethyl, 2-aminoethyl, 2,2-diaminoethyl, 2-aminoisopropyl, 5-aminopentyl, 1,2-aminododecyl, 1,2-diaminoethyl, 1,5-diaminopentyl, aminocyclobutyl, aminocyclohexyl, 3-amino-1-propen-1-yl, 5-amino-2-penten-1-yl, aminophenyl, (methylamino)phenyl, 2-amino-o-tolyl, 4-amino-m-tolyl, 3-amino-p-tolyl, and other positional isomers, various isomers of diaminophenyl, amino-2,5-xylyl, and various positional isomers thereof, 2-amino-1-naphthyl, 3-amino-1-naphthyl, 2-amino-3-methyl-1-naphthyl, 2,3-diamino-5-ethyl-1-naphthyl, and the like.

The R groups may contain amide groups which may be illustrated by such non-limiting examples as: carbamoylmethyl, 2-carbamoylethyl, 4-carbamoylbutyl, 8-carbamoyl-2-ethyloctyl, 1,4-dicarbamoylbutyl, carbamoylcyclopentyl, carbamoylcyclohexyl, 2-carbamoyl-o-tolyl, 2-carbamoyl-m-tolyl, 3-carbamoyl-p-tolyl, (carbamoylmethyl)phenyl, (2-carbamoylethyl)benzyl; o, m, and p-(carbamoylethyl)phenyl, and the like.

The preferred hydrocarbys are the alkyls, especially the lower alkyls having from 1 to about 10 carbon atoms, with the more preferred alkyls being ethyl and methyl. The most preferred alkyl is ethyl.

While the preferred antiplugging compounds of the present invention have the general formula



with the most preferred antiplugging compound having the formula



it is to be understood that the scope of the present invention contemplates compounds having the general formula



with R as defined above and R<sub>1</sub>, R<sub>2</sub> and R<sub>3</sub> being independently selected from hydrogen, hydrocarbyl radi-

cals of up to 10 carbon atoms, and substituted hydrocarbyl radicals of up to 10 carbon atoms.

Some non-limiting representative examples of these hydrocarbyl radicals are alkyl, cycloalkyl, alkenyl, aralkyl, alkaryl, and aryl.

Examples of alkyl groups represented by R<sub>1</sub>, R<sub>2</sub> and R<sub>3</sub> in the above general formula are methyl, ethyl, n-propyl, isopropyl, n-butyl, isobutyl, sec-butyl, tert-butyl, n-amyl, and the various positional isomers thereof, and likewise the corresponding straight and branched chain isomers of hexyl, heptyl, octyl, nonyl, decyl, undecyl, dodecyl, and the like.

Examples of cycloalkyl groups are cyclopropyl, cyclobutyl, cyclopentyl, cyclohexyl, cycloheptyl, cyclooctyl, cyclononyl, and cyclodecyl.

The R<sub>1</sub>, R<sub>2</sub> and R<sub>3</sub> groups in the above general formula may also be alkenyl groups such as ethenyl, 1-propenyl, 2-propenyl, isopropenyl, 1-butenyl, 2-butenyl, 3-butenyl, and the corresponding branched-chain isomers thereof as for example, 1-isobut enyl, 2-isobut enyl, 2-sec-but enyl, including 1-methylene-2-propenyl, and the various isomers of pentenyl, hexenyl, heptenyl, octenyl, nonenyl, and decenyl, including 2,3-dimethyl-2-but enyl, 2,3-dimethyl-3-but enyl, 1-methyl-1-ethyl-2-propenyl, and the like.

When said R<sub>1</sub>, R<sub>2</sub> and R<sub>3</sub> groups are alkaryl groups, they may be tolyl, 2,3-xylyl, 2,4-xylyl, 2,5-xylyl, 2,6-xylyl, 3,4-xylyl, and 3,5-xylyl.

Phenyl is an aryl group which may be present in the above general formula.

When said R<sub>1</sub>, R<sub>2</sub> and R<sub>3</sub> groups are aralkyl groups, they may be benzyl, phenylethyl, 1-phenylpropyl, 2-phenylpropyl, 3-phenylpropyl, 1- and 2-isomers of phenylisopropyl, 1-, 2-, and 3-isomers of phenylbutyl, and the like.

The substituted hydrocarbyl radicals are hydrocarbyl radicals which contain substituents such as halogen, hydroxyl, carboxyl, alkoxy carbonyl, amino, or amide radicals. Thus, the R<sub>1</sub>, R<sub>2</sub> and R<sub>3</sub> groups may contain the same or different substituents or any one of the R<sub>1</sub>, R<sub>2</sub> and R<sub>3</sub> groups may contain one or more of said radicals substituted thereon.

As mentioned above, the R<sub>1</sub>, R<sub>2</sub> and R<sub>3</sub> groups may be halogen substituted. Thus, chlorine, bromine, iodine, and fluorine may be substituted on the alkyl, cycloalkyl, alkenyl, alkaryl, aryl, and aralkyl groups which are present. Non-limiting examples of such substituted groups are chloromethyl, cyanoethyl, bromoethyl, 2-fluoro-1,2-dibromoethyl, 1-iodopropyl, 2-fluoropropyl, 1-chlorobutyl, 2-bromobutyl, 2-iodo-2-methylpropyl, 1-chloropentyl, 3-fluoro-2-methylbutyl, 3-iodo-2-methylbutyl, 1-chloro-2,2-dimethylpropyl, 2-chloroheptyl, 3-fluorononyl, 1-chlorododecyl, and the like. Examples of halogenated cycloalkyl groups are chlorocyclopropyl, chlorocyclohexyl, 1,2-dichlorohehexyl, bromocyclobutyl, iodocyclohexyl, and the like.

Examples of halogen-substituted alkenyl groups are bromoethenyl, chloroethenyl, iodoethenyl, 1-bromododecyl, and the like.

Examples of halogenated alkaryl groups are chloro-o-tolyl, chloro-p-tolyl, chloro-m-tolyl, 2-bromo-3,4-xylyl, 4-bromo-2,3-xylyl, 5-bromo-2,4-xylyl, 2-bromo-4,5-xylyl, o, m, and p-tolyl, and the like.

Examples of halogen substituted aryl groups are bromophenyl, 2,4-dibromophenyl, 2,3-dibromophenyl, 2,5-dibromophenyl, 2,3,4,5-tetrabromophenyl, 2,3,5,6-tetra-

bromophenyl, pentabromophenyl, and all isomers of chlorophenyl.

Amine groups may also be substituted on the R<sub>1</sub>, R<sub>2</sub> and R<sub>3</sub> groups. Some non-limiting illustrative examples of R<sub>1</sub>, R<sub>2</sub> and R<sub>3</sub> groups containing amine substituents are aminomethyl, 2-aminoethyl, 2,2-diaminoethyl, 2-aminoisopropyl, 5-aminopentyl, 1,2-diaminoethyl, 1,5-diaminopentyl, aminocyclobutyl, aminocyclohexyl, 2-amino-o-tolyl, 4-amino-m-tolyl, 3-amino-p-tolyl, and other positional isomers, various isomers of 10 diaminophenyl, amino-2,5-xylyl, and various positional isomers thereof, and the like.

The R<sub>1</sub>, R<sub>2</sub> and R<sub>3</sub> groups may contain amide groups which may be illustrated by such non-limiting examples as: carbamoylmethyl, 2-carbamoylethyl, 4-carbamoylbutyl, 8-carbamoyl-2-ethyloctyl, 1,4-dicarbamoylbutyl, carbamoylcyclopentyl, carbamoylcyclohexyl, 2-carbamoyl-o-tolyl, 2-carbamoyl-m-tolyl, 3-carbamoyl-p-tolyl, (carbamoylmethyl)phenyl, (2-carbamoylethyl)-benzyl; o, m, and p-(carbamoylethyl)phenyl, and the like.

The preferred hydrocarbys are the alkyls, preferably the lower alkyls, and most preferably the lower alkyls having from 1 to about 5 carbon atoms. The preferred esters are the trialkyl esters of 1,1,2-ethane tricarboxylic acid such as the trimethyl, triethyl, tripropyl, tributyl, trioctyl, and tridecyl esters or mixtures of two or more such esters, with the most preferred esters being triethyl 1,1,2-ethane tricarboxylate. In order to be most advantageously employed as antiplugging agents, the above compounds should be readily soluble, either directly or indirectly, in the gasoline.

15 1,1,2-Ethane tricarboxylic acid and its esters, particularly the lower alkyl esters, are known compounds whose preparation is known in the art.

20 Of the compounds having the general formula



25 compounds wherein R, R<sub>1</sub>, R<sub>2</sub> and R<sub>3</sub> are independently selected from hydrogen and hydrocarbyl radicals are preferred. The preferred hydrocarbyl radicals are those containing up to 10 carbon atoms, more preferred hydrocarbyl radicals are alkyl radicals containing up to 10 carbon atoms.

30 Tests were run to illustrate the unusual and beneficial effects of one compound of this invention on reducing exhaust catalyst plugging with manganese. In such tests a single cylinder engine was used. The A/F mixture was held at approximately 16.0:1 maintaining 1.8% oxygen in the exhaust stream. The engine speed was run generally with a wide open throttle with the spark firing at an appropriate crank angle, depending on engine characteristics and exhaust gas temperature required.

35 Generally an exhaust gas temperature range of from 1,500° F. to 1,700° F. in the catalyst entrance cone was maintained.

40 The exhaust catalysts used were PTX units manufactured and sold by Engelhard Industries. The particular PTX unit used was the PTX-3 which is composed of a cordierite ceramic core which has a random stacked, 16 cell/inch configuration. The ceramic has 0.2 wt. percent platinum with 0.5 g Pt on the entire ceramic core of the PTX-3 unit. This ceramic is 2.625 inches in diameter, 3.8 inches long and is encased in a Monel mesh to

take care of thermal expansion differences between the ceramic and steel housing. This is encased in a stainless steel housing 3 inches outer diameter and 4 inches long. The ceramic is held firmly in place by two retaining rings on the face of the ceramic welded to the steel casing; in addition 1/4 inch square strips are welded to the casing to prevent rotation of the core. The inlet and outlet cover of the unit are 1.5 inches long and the sides form a 45° angle. The casings are joined to a pipe which is connected to the exhaust system. A standard unleaded gasoline of the type described above was used with 1.0 g Mn/gal as methylcyclopentadienyl manganese tricarbonyl. The concentration of triethyl ester added to the 45 gasoline was 0.2 g/gal. To determine when the PTX-3 unit was plugged the back pressure in the exhaust stream in front of the PTX-3 unit was measured at predetermined intervals, usually every one or two hours, as the test progressed. The initial back pressure readings generally varied from 0.2 to 0.6 psi. When the back pressure reached a value of 2.0 psi the system was considered plugged and the test was terminated.

50 The following results were obtained in the above tests when triethyl 1,1,2-ethane tricarboxylate was used in the test fuel.

TABLE II

| Temp.    | Mn conc.         | Triethyl<br>1,1,2-ethane<br>tricarboxylate<br>conc. | Hours to plug                                                  |
|----------|------------------|-----------------------------------------------------|----------------------------------------------------------------|
| 1500° F. | 1g/gal<br>1g/gal | 0<br>0.2g/gal                                       | 45<br>at 197 hours<br>the catalyst<br>was about<br>30% plugged |
|          |                  |                                                     |                                                                |

55 The test was terminated at 197 hours. At this point the catalyst was about 30% plugged, by surface area. The back pressure reading at 197 hours was about 1.25 psi.

60 The amount of antiplugging compound, as for example, triethyl 1,1,2-ethane tricarboxylate, sufficient to reduce the plugging of the catalyst is at least to some extent dependent upon the amount of manganese present in the gasoline and on the inlet exhaust temperature. Generally, the greater the concentration of manganese and the higher the temperature the greater the amount of antiplugging compound needed to reduce plugging of the catalyst.

65 The lower limit at which the antiplugging compounds of the present invention, such as triethyl 1,1,2-ethane tricarboxylate, are effective to reduce plugging is about 0.01 g/gal. Preferably, the amount of the compound is greater than 0.03 g/gal, and more preferably greater than 0.125 g/gal. There is no real upper limit on the concentration of the antiplugging compound, and, accordingly, the upper limit is restricted by such secondary considerations as economics, etc. Therefore, since the amount of the antiplugging compound, such as the aforementioned triethyl ester, is quite dependent upon the concentration of the manganese, for practical purposes the upper limit is about 10 g/gal. Generally, the amount of antiplugging compound present in the gasoline should be an amount effective to reduce the plugging of the catalyst. In addition to being hydrogen, hydrocarbyl radicals, and substituted hydrocarbyl radicals the R groups in the general formulae



may also be ammonium and substituted ammonium cations such as morpholinium, alkyl ammonium and mono-, di-, and trialkanol ammonium.

Corresponding esters wherein from 1 to 2 of the ammonium and/or substituted ammonium cations are replaced with organic groups can also be used. Typical organic groups include the aforementioned hydrocarbyl and substituted hydrocarbyl radicals. Thus two of the R groups can be ammonium or ammonium cations while one of the R groups can be said aforementioned organic group; one of the R groups can be an ammonium or substituted ammonium cation, one R group can be hydrogen, and one R group can be said organic group; one R group can be a metal cation, one R group can be an ammonium or substituted ammonium cation, and one R group can be an organic group; or two R groups can be organic groups and the other R group can be an ammonium or substituted ammonium cations.

It is convenient to utilize additive fluid mixtures which consist of cyclopentadienyl manganese tricarbonyl antiknock agents and antiplugging agents having the general formula



and the preferred formula



wherein R, R<sub>1</sub>, R<sub>2</sub> and R<sub>3</sub> are as defined above. These additive fluid mixtures are added to low-lead or unleaded gasoline. In other words, part of the present invention are antiknock-antiplugs fluids which comprise cyclopentadienyl manganese tricarbonyl antiknock agents and the antiplugging agents of the type described hereinabove.

Use of such antiknock-antiplugs fluids in addition to resulting in great convenience in storage, handling, transportation, blending with fuels, and so forth, also are potent concentrates which serve the multipurpose functions of being useful as antiknocks and catalyst plugging reducers.

In these fluid compositions the weight ratio of manganese-to-antiplugging agents can vary from about 0.03 gram of an antiplugging agent such as triethyl 1,1,2-ethane tricarboxylate to 1 gram of manganese or even 0.01 gram of the antiplugging agent such as triethyl 1,1,2-ethane triethyl 1,1,2-ethane tricarboxylate to 1 gram of manganese on the one hand to about 10 grams of the antiplugging agent such as triethyl 1,1,2-ethane tricarboxylate to about 1 gram of manganese on the other hand. Some typical preferred fluids are those containing a ratio of 0.03 grams of triethyl 1,1,2-ethane tricarboxylate to 0.125 grams of manganese, 0.06 grams of triethyl 1,1,2-ethane tricarboxylate to 0.125 grams of manga-

5

nese, 0.2 gram of triethyl 1,1,2-ethane tricarboxylate to 1 gram of manganese, 0.1 gram of triethyl 1,1,2-ethane tricarboxylate to 0.25 gram of manganese, 0.5 gram of triethyl 1,1,2-ethane tricarboxylate to 1 gram of manganese, and 1 gram of triethyl 1,1,2-ethane tricarboxylate to 1 gram of manganese. The fluids may optionally contain other additives such as antioxidants, antirust agents, detergents, etc., as well as solvents, e.g., hydrocarbon, to facilitate handling.

Although generally the antiplugging compounds of the present invention have the general formula



wherein R, R<sub>1</sub>, R<sub>2</sub> and R<sub>3</sub> have been previously described, it is believed that compounds having the skeletal structure



25

will have useful properties in reducing the plugging of exhaust catalysts.

30

It is also believed that compounds of the type generally described as tricarbalkoxy hydrocarbons will generally also have useful properties in reducing the plugging of exhaust catalysts. By tricarbalkoxy hydrocarbon is meant a hydrocarbon to which are attached three carbalkoxy, —COOR groups, wherein R is a hydrocarbyl radical, preferably a hydrocarbyl radical of up to about 10 carbon atoms, and more preferably an alkyl radical of up to about 10 carbon atoms. Examples of suitable hydrocarbyl radicals are set forth above. For purposes of the present invention a hydrocarbon can be defined as an organic group composed solely of hydrogen and carbon atoms. Some non-limiting representative examples of hydrocarbons are the alkyls, cycloalkyls, alkenyls, aralkyls, alkaryl, and aryls. The preferred hydrocarbons are the trivalent hydrocarbons. The preferred trivalent hydrocarbons are those having up to about 10 carbon atoms. Thus, preferred trivalent hydrocarbons can be trivalent alkyls, cycloalkyls, alkenyls, aralkyls, alkaryl, and aryls having up to about 10 carbon atoms, more preferably 2 to 10 carbon atoms.

35

Examples of alkyl groups having up to about 10 carbon atoms are methyl, ethyl, n-propyl, isopropyl, n-butyl, isobutyl, sec-butyl, tert-butyl, n-amyl, and the various positional isomers thereof, and likewise the corresponding straight and branched chain isomers of hexyl, heptyl, octyl, nonyl, and decyl.

40

Examples of cycloalkyl groups having up to about 10 carbon atoms are cyclopropyl, cyclobutyl, cyclopentyl, cyclohexyl, cycloheptyl, cyclooctyl, cyclononyl, and cyclodecyl.

45

Examples of alkenyl groups having up to about 10 carbon atoms are ethenyl, 1-propenyl, 2-propenyl, isopropenyl, 1-butenyl, 2-butenyl, 3-butenyl, and the corresponding branched-chain isomers thereof as for example, 1-isobutenyl, 2-isobutenyl, 2-sec-butenyl, including 1-methylene-2-propenyl, and the various isomers of pentenyl, hexenyl, heptenyl, octenyl, nonenyl, and decenyl.

Examples of alkaryl groups having up to about 10 carbon atoms are tolyl, 2,3-xylyl, 2,4-xylyl, 2,5-xylyl, 2,6-xylyl, 3,4-xylyl and 3,5-xylyl.

Examples of aralkyl groups having up to about 10 carbon atoms are benzyl, phenylethyl, 1-phenylpropyl, 2-phenylpropyl, 3-phenylpropyl, 1- and 2-isomers of phenylisopropyl, 1-, 2-, and 3-isomers of phenylbutyl, and the like.

The more preferred trivalent hydrocarbons are the trivalent alkyls having up to about 10 carbon atoms, with the trivalent alkyls having from 2 to 10 carbon atoms being most preferred.

The three carbalkoxy groups,  $-\text{COOR}$  wherein R is a hydrocarbyl group, preferably a hydrocarbyl group of up to about 10 carbon atoms, and more preferably an alkyl group of up to about 10 carbon atoms, can be substituted (1) on the same carbon atom in the trivalent hydrocarbon, (2) upon three different carbon atoms in the trivalent hydrocarbon, (3) or two carbalkoxy groups can be substituted on one carbon atom in the trivalent hydrocarbon while the third carbalkoxy group is substituted on a second carbon atom in the trivalent hydrocarbon. Thus, for example, triethyl 1,1,2-ethane tricarboxylate



falls within the class of trivalent hydrocarbons defined as (3) above, that is, wherein two carbalkoxy groups are substituted upon one carbon atom in the hydrocarbon radical while the third carbalkoxy group is substituted upon the second carbon atom in the hydrocarbon radical.

The aforementioned tricarbalkoxy hydrocarbons have the general formula



wherein R' is a trivalent hydrocarbon radical, preferably one containing 1 to about 10 carbon atoms, more preferably containing 2 to about 10 carbon atoms, and most preferably an alkyl group containing 2 to about 10 carbon atoms, and wherein each R is independently selected from hydrocarbyl radicals, preferably hydrocarbyl radicals containing 1 to about 10 carbon atoms, and more preferably alkyl radicals containing 1 to about 10 carbon atoms.

Some non-limiting representative examples of trivalent hydrocarbon radicals are trivalent alkyl, trivalent cycloalkyl, trivalent alkenyl, trivalent aralkyl, trivalent alkaryl, and trivalent aryl radicals.

Preferred trivalent hydrocarbon radicals are those containing up to about 10 carbon atoms. More preferred trivalent hydrocarbon radicals are those containing from 2 to about 10 carbon atoms. Most preferred trivalent hydrocarbon radicals are trivalent alkyl radicals containing from 2 to about 10 carbon atoms.

Some examples of trivalent hydrocarbon radicals containing 2 to 10 carbon atoms are set forth below



Thus another embodiment of the present invention is a gasoline composition comprising (i) an antiknock amount of a cyclopentadienyl manganese tricarbonyl antiknock, and (ii) an amount effective to reduce the plugging of an exhaust gas catalyst of a compound having the general formula



10

wherein  $\text{R}'$  is a trivalent hydrocarbon radical, and wherein each  $\text{R}$  is independently selected from hydrocarbyl radicals. Preferably  $\text{R}'$  is a trivalent hydrocarbon radical containing from 1 to about 10 carbon atoms, more preferably from 2 to about 10 carbon atoms, and most preferably an alkyl radical containing from 2 to about 10 carbon atoms.

Yet another embodiment of the present invention is an additive fluid composition for gasoline comprising (i) a cyclopentadienyl manganese tricarbonyl antiknock, and (ii) a compound having the general formula



wherein  $\text{R}'$  is a trivalent hydrocarbon radical and  $\text{R}$  is independently selected from hydrocarbyl radicals. Preferably  $\text{R}'$  is a trivalent hydrocarbon radical containing from 1 to about 10 carbon atoms, more preferably from 2 to about 10 carbon atoms, and most preferably an alkyl radical containing from 2 to about 10 carbon atoms.

Claims to the invention follow.

I claim:

1. A gasoline composition for a spark ignited internal combustion engine comprising
  - i. an antiknock amount of a cyclopentadienyl manganese tricarbonyl antiknock, and
  - ii. an amount effective to reduce the plugging of an exhaust gas catalyst of a compound having the general formula



35

wherein  $\text{R}$ ,  $\text{R}_1$ ,  $\text{R}_2$  and  $\text{R}_3$  are independently selected from hydrogen, hydrocarbyl and substituted hydrocarbyl radicals.

2. The composition of claim 1 wherein said cyclopentadienyl is a hydrocarbon group having from 5 to 17 carbon atoms.

3. The composition of claim 2 wherein said cyclopentadienyl is methylcyclopentadienyl.

4. The composition of claim 3 wherein  $\text{R}_1$ ,  $\text{R}_2$  and  $\text{R}_3$  are independently selected from hydrogen and hydrocarbyl radicals and wherein  $\text{R}$  is independently selected from hydrocarbyl radicals.

5. The composition of claim 4 wherein  $\text{R}_1$ ,  $\text{R}_2$  and  $\text{R}_3$  are independently selected from hydrogen and alkyl radicals and wherein  $\text{R}$  is independently selected from alkyl radicals.

6. The composition of claim 5 wherein said alkyl radicals are lower alkyl radicals.

7. An additive fluid composition for gasoline comprising

- i. a cyclopentadienyl manganese tricarbonyl antiknock, and
- ii. a compound having the general formula



wherein  $\text{R}$ ,  $\text{R}_1$ ,  $\text{R}_2$  and  $\text{R}_3$  are independently selected from hydrogen, hydrocarbyl, and substituted hydrocarbyl radicals.

8. The composition of claim 7 wherein said cyclopentadienyl is hydrocarbon group having from 5 to 17 carbon atoms.

9. The composition of claim 8 wherein said cyclopentadienyl is methylcyclopentadienyl.

10. The composition of claim 9 wherein  $\text{R}_1$ ,  $\text{R}_2$  and  $\text{R}_3$  are independently selected from hydrogen and hydrocarbyl radicals and wherein  $\text{R}$  is independently selected from hydrocarbyl radicals.

11. The composition of claim 10 wherein said hydrocarbyl radicals are alkyl radicals.

12. The composition of claim 11 wherein said alkyl radicals are lower alkyl radicals.

13. A gasoline composition for a spark ignited internal combustion engine comprising

- i. an antiknock amount of a cyclopentadienyl manganese tricarbonyl antiknock, and
- ii. an amount effective to reduce the plugging of an exhaust gas catalyst of a compound having the general formula



wherein  $\text{R}$  is independently selected from hydrogen and hydrocarbyl radicals.

14. A gasoline composition of claim 13 wherein said cyclopentadienyl is a hydrocarbon group having from 5 to 17 carbon atoms.

15. The composition of claim 14 wherein said cyclopentadienyl is methylcyclopentadienyl.

16. The composition of claim 14 wherein  $\text{R}$  is independently selected from hydrocarbyl radicals.

17. The composition of claim 16 wherein said hydrocarbyl radicals are alkyl radicals.

18. The composition of claim 17 wherein said alkyl radicals are lower alkyl radicals.

19. The composition of claim 18 wherein each  $\text{R}$  is ethyl.

20. An additive fluid composition for gasoline comprising

- i. a cyclopentadienyl manganese tricarbonyl antiknock, and
- ii. a compound having the general formula



wherein R is independently selected from hydrogen and hydrocarbyl radicals.

21. The composition of claim 20 wherein said cyclopentadienyl is a hydrocarbon group having from 5 to 17 carbon atoms.

22. The composition of claim 21 wherein said cyclopentadienyl is methylcyclopentadienyl.

23. The composition of claim 22 wherein R is independently selected from hydrocarbyl radicals.

24. The composition of claim 23 wherein said hydrocarbyl radicals are alkyl radicals.

25. The composition of claim 24 wherein said alkyl radicals are lower alkyl radicals.

26. The composition of claim 25 wherein each R is ethyl.

27. A low-lead or essentially lead-free gasoline composition for a spark ignited internal combustion engine comprising

i. an amount effective to improve the antiknock properties of said gasoline composition of a cyclopentadienyl manganese tricarbonyl antiknock, and

ii. an amount effective to reduce the plugging of an exhaust gas catalyst of a compound having the general formula



wherein R is independently selected from hydrogen and hydrocarbyl radicals.

28. The composition of claim 27 wherein said cyclopentadienyl is a hydrocarbon group having from 5 to 17 carbon atoms.

29. The composition of claim 28 wherein said cyclopentadienyl is methylcyclopentadienyl.

30. The composition of claim 29 wherein R is independently selected from a hydrocarbyl radical.

31. The composition of claim 30 wherein said hydrocarbyl radical is an alkyl radical.

32. The composition of claim 31 wherein said alkyl radical is a lower alkyl radical.

33. The composition of claim 32 wherein each R is ethyl.

34. An additive fluid concentrate for lead-free or essentially lead-free gasoline comprising

i. a cyclopentadienyl manganese tricarbonyl anti-knock, and

ii. a compound having the general formula



wherein R is independently selected from hydrogen and hydrocarbyl radicals.

35. The concentrate of claim 34 wherein said cyclopentadienyl is a hydrocarbon group having from 5 to 17 carbon atoms.

36. The concentrate of claim 35 wherein said cyclopentadienyl is methylcyclopentadienyl.

37. The concentrate of claim 36 wherein R is independently selected from hydrocarbyl radicals.

38. The concentrate of claim 37 wherein said hydrocarbyl radicals are alkyl radicals.

39. The concentrate of claim 38 wherein said alkyl radicals are lower alkyl radicals.

40. The concentrate of claim 39 wherein each R is ethyl.

\* \* \* \* \*